

FIP8309 XR 1,217,744  
LAIUN OF TEXTILES & FIBERS,

## UNITED STATES PATENT OFFICE.

ALBERT E. GARRETT, OF YAVERLAND, ST. ALBANS, ENGLAND.

## PROCESS FOR PRODUCING WHITE WOOLEN GOODS.

1,217,744.

Specification of Letters Patent.

Patented Feb. 27, 1917.

No Drawing.

Application filed August 30, 1916. Serial No. 117,676.

*To all whom it may concern:*

Be it known that I, ALBERT EDWARD GARRETT, a subject of the King of Great Britain, and resident of Yaverland, Clarence 5 Road, St. Albans, in the county of Hertford, England, analyst, have invented a certain new and useful Improved Process for Producing White Woolen Goods, of which the following is a specification.

10 This invention relates to the production of white woolen goods. Various methods are known of bleaching woolen goods, and one of these methods is to use hydrogen peroxid, with or without subsequent "stoving" 15 of the goods with sulfur dioxid. Hitherto, this method of bleaching has not found much favor as it is slow and expensive to apply, and unless great care is taken the goods are liable to be irregularly 20 bleached, giving a blotchy appearance. Hence, the bleaching methods most generally employed have been those using reducing agents, but they are not by any means permanent, and the goods are liable to return 25 to their natural color after washing a few times.

It is the object of the present invention to effect the bleaching by an oxidizing method using hydrogen peroxid, but the treatment 30 is accelerated and the result attained with certainty by the use of a subsequent treatment in a weak ammonia bath having for its object to decompose the hydrogen peroxid quickly on the goods with the formation of 35 nascent oxygen, this being the essential bleaching agent.

The following example will indicate the application of the process according to the present invention, to the production of white 40 woolen goods such as underwear.

The goods are first scoured and may then be rendered unshrinkable by treatment in a chlorin bath in the known manner, if this is desired. After the chlorination the goods 45 are scoured in order to remove superfluous chemical reagents. A weak bath of hydrogen peroxid is prepared, and although the strength of this bath may vary, it will never contain more than 1% of  $H_2O_2$ ; 10-volume- 50 strength hydrogen peroxid contains about 3% of  $H_2O_2$ , and by way of example it may be mentioned that a 10 per cent. solution of 10-volume-strength hydrogen peroxid (containing therefore about 0.3% of 55  $H_2O_2$ ) has given satisfactory results in prac-

tice. The bath is kept at a luke-warm temperature, and at any rate not higher than 50° C., the goods being steeped in the bath for a few minutes until they are thoroughly saturated with the solution. They are then 60 squeezed out and immersed at once in another bath containing a weak solution of ammonia. As an example of the strength of this bath, it may be mentioned that 4 or 5 cubic centimeters of concentrated (0.880) 65 ammonia per liter of water at 50° centigrade will give good results. To this bath may also be added four or five grams of a pure soap per liter, the function of the soap probably being to act as a detergent in order to permit the ammonia to be fully utilized in reacting with the hydrogen peroxid. The goods are not left in the ammonia bath but are merely dipped into it to saturate 70 them with the ammonia solution, and are then squeezed out at once. They are hung up to dry for any suitable period of time, say from one to two hours, and during this period the ammonia remaining on the goods reacts with the hydrogen peroxid thereon, 75 causing oxygen to be released in the nascent state and to effect the bleaching action. When this has taken place to a satisfactory extent, the goods are cleared in a thorough manner and finally scoured, dried and 80 finished by pressing.

By the use of the ammonia bath according to this invention, the action of the hydrogen peroxid is greatly accelerated and the result attained is more satisfactory than 90 that obtainable by any other known process of bleaching using an oxidizing agent. After the bleaching with peroxid as above set forth, the whiteness of the goods is rather improved than otherwise by subsequent 95 washing, so that the bleach can be regarded as a permanent one.

The goods may be stoved if desired after the bleaching with peroxid, and after they have been cleared but before the final scouring, drying and finishing. It is found that stoving at this stage for a short time (in sulfur dioxid), gives a rather brighter white than can be attained by the peroxid bleaching alone, but the white will probably 105 not be so permanent as a rule after stoving. It may be sufficiently permanent however for practical purposes, and the oxidizing-bleaching action produced by the peroxid is not destroyed by stoving at this stage. 110

Having thus described my invention what I claim as new and desire to secure by Letters Patent is:—

1. A process of bleaching white woolen goods consisting in immersing such goods in a weak solution of hydrogen peroxid, squeezing out the goods, dipping them in a weak ammonia solution, squeezing out the goods again, and hanging them up for a period during which a reaction of the ammonia with the hydrogen peroxid takes place.
2. A process of bleaching white woolen goods consisting in immersing such goods in a weak solution of hydrogen peroxid not exceeding a strength of 1 per cent., squeezing out the goods, dipping them in a weak ammonia solution, squeezing out the goods again, and hanging them up for a period during which a reaction of the ammonia with the hydrogen peroxid takes place.
3. A process of bleaching white woolen goods consisting in immersing such goods in a weak solution of hydrogen peroxid, squeezing out the goods, dipping them in a weak ammonia solution containing approximately 5 cubic centimeters of concentrated ammonia per liter of water and maintained at approxi-

mately 50° C., squeezing out the goods again, and hanging them up for a period during which a reaction of the ammonia with the hydrogen peroxid takes place.

4. A process of bleaching white woolen goods consisting in immersing such goods in a weak solution of hydrogen peroxid, squeezing out the goods, dipping them in a weak ammonia solution to which is added approximately 5 grams of pure soap per liter of solution, squeezing out the goods again, and hanging them up for a period during which a reaction of the ammonia with the hydrogen peroxid takes place.

5. A process of bleaching white woolen goods consisting in immersing such goods in a weak solution of hydrogen peroxid, squeezing out the goods, dipping them in a weak ammonia solution containing approximately 5 cubic centimeters of concentrated ammonia per liter of water and approximately 5 grams of pure soap per liter and maintained at approximately 50° C., squeezing out the goods, and hanging them up for a period during which a reaction of the ammonia with the hydrogen peroxid takes place.

ALBERT E. GARRETT.